

March 2, 1954

W. L. BOSTWICK ET AL

2,670,555

CARRIER-BACKED DECORATIVE MATERIAL

Filed Nov. 2, 1950



Fig. 1



Fig. 2

INVENTORS.

Wallace L. Bostwick  
Samuel M. Terry

BY Adams, Stevens & Mase

AGENTS.

## UNITED STATES PATENT OFFICE

2,670,555

## CARRIER-BACKED DECORATIVE MATERIAL

Wallace L. Bostwick and Samuel M. Terry, Columbus, Ohio, assignors, by mesne assignments, to The United States Playing Card Company, Cincinnati, Ohio, a corporation of Ohio, and National Publishing Company, Philadelphia, Pa., a corporation of Pennsylvania

Application November 2, 1950, Serial No. 193,668

8 Claims. (Cl. 41—37)

1

This invention relates to a carrier-backed decorating material and, more particularly, to a carrier-backed decorating material having incorporated therewith a material for preventing abrasion of the decorative film.

Decorated surfaces, such as embossed surfaces, or the flat surfaces formed by a plurality of edge-decorated book sheet edges or card edges, lose their lustrous appearance, become dull, and disintegrate mainly through the action of abrasive forces. This is particularly true in the case of edge-decorated book sheets or playing cards when merely subjected to the abrasion attendant upon their normal use. In the past, attempts have been made to solve this problem by providing a layer of a protective material, so positioned in the carrier-backed decorative strip, that upon application of the strip to the surface formed from a plurality of card edges or sheet edges, or any other flat surface, such as a flat leather surface, or the like, the protective coating layer would be exposed to the abrasive forces, and would be positioned exterior of the decorative material. In other words, the resultant decorated surface would comprise a layer of adhesive, contacting the flat surface, and also contacting the decorative material, and a layer of the protective material, exterior of the decorative material. Such exteriorly positioned protective materials have been unsatisfactory since, while offering some protection to the decorative material, they have detracted from the lustrous appearance of the decorated surface and, consequently, have decreased the sales appeal of the particular item in question. Most of these substances, moreover, upon aging, have become more opaque, thereby even further detracting from the pleasing appearance of the decorated article. In the book sheet edge-decorating and playing card edge-decorating arts, it was originally the practice to decorate the flat surface formed by a plurality of book sheet edges or playing card edges with a thin metallic leaf such as gold, silver, or the like, by first cleaning and otherwise preparing the surface, applying adhesive thereto, and then applying the unsupported leaf to the adhesively treated surface. At the proper instant, the decorative material was burnished by a highly skilled workman and then, if desired, a layer of a protective coating material was placed on the decorated surface. The entire procedure was extremely expensive, and where the protective coating material became discolored, upon aging, there resulted an article of manufacture so lacking in sales appeal, that in both of these arts the

2

practice has been, in the majority of instances, not to include the use of a protective coating material.

It is, therefore, one object of this invention to provide a carrier-backed decorative strip wherein the decorative material will be rendered resistant to abrasion when placed on a surface and at the same time will present a lustrous appearance.

It is another object of this invention to provide an edge-decorated book sheet, playing card, or the like, wherein the decorative material is resistant to abrasion.

It is still another object of this invention to provide the edge-decorated book sheet, playing card, or the like, wherein the decorative material is bonded to the edge of the book sheet, playing card, or the like, by means of a heat-activated adhesive, and wherein the decorative material is rendered resistant to abrasion.

It is a further object of this invention to provide a material for decorating the edges of book sheets, playing cards, or the like, which is simple to use, inexpensive, and which will permit the decoration of all of the exposed edges of a group of book sheets, playing cards, or the like, assembled en masse, all in one operation, and which will minimize the abrasion of the decorative material when that decorative material has been applied to the edges of book sheets, playing cards, or the like.

Various other objects and advantageous features of this invention may be had from the following description when read in conjunction with the accompanying drawings, in which

Fig. 1 is a fragmentary, perspective view of a carrier-backed decorative strip, the individual parts thereof being exaggerated in size for purposes of clarity; and

Fig. 2 is a fragmentary side elevation view, partly in section, of an edge-decorated book sheet or playing card.

In general, this invention is based upon the discovery that the incorporation of a particular material in admixture with an adhesive, in a layer which contacts both the decorative material and the adhesive material, results in a carrier-backed decorative strip which, when applied to a flat surface, or the edge of a playing card, book sheet, or the like, will protect the decorative material from wear due to abrasion, even though the decorative material is exposed to the abrasive forces, and does not have a protective coating material thereover.

Referring to the drawings, and, more partic-

ularly, to Fig. 1, a carrier-backing 10 of a suitable material, such as cellophane, paper, or the like, has applied thereto a film or coating of release material 11. This film of release material may be applied in a variety of ways, vacuum evaporation being a very satisfactory method for insuring the production of a film of uniform, controlled thickness. Substantially the only requirements for the backing strip are that it be flexible, have a smooth surface, and be substantially nonelastic. Waxes and alkali halide salts such as potassium bromide (KBr) or potassium iodide (KI), are good release materials. 12 is a film of decorative material, such as gold, silver, aluminum, brass, bronze, or the like. This film of decorative material may be applied to the release material by vacuum evaporation, sputtering, or any other satisfactory method. Layer 13 is a mixture of nitrocellulose and an adhesive, and layer 14 is an adhesive.

It is preferred that the adhesive be a heat-activated type of adhesive, and, more particularly, it is preferred that the heat-activated type of adhesive be a polyamide adhesive. Polyamide adhesives formed from ethylene diamine and dimerized, trimerized linoleic and linolenic acids have proven very successful as heat-activated polyamide type adhesives. It is preferred that layer 13 contain from approximately 25% to approximately 70% nitrocellulose, the balance being polyamide adhesive. Below approximately 25% inclusion of nitrocellulose in layer 13 there is no noticeable improvement in abrasion-resistant qualities, as compared to a decorative material adhered to a surface merely by means of a polyamide adhesive. More than 70% nitrocellulose results in such an increase in the cohesion of layer 13 that, when the carrier-backed decorative material has been applied to the surface formed by the edges of book sheets or playing cards, the individual pages of books or the individual playing cards cannot be readily separated from each other without damage to the decorated surface. In a case of the embossing of a flat surface, such as leather, or the like, more than 70% nitrocellulose in layer 13 results in such an increase in the cohesion of the layer that the lines of demarcation of the embossed areas are frequently ragged, thereby producing an unsatisfactory article.

The most preferred composition of layer 13 is 50% nitrocellulose and 50% polyamide adhesive.

Any of the soluble types of nitrocellulose may be used. Included within such a category are the RS, AS, and SS types of nitrocellulose. While nitrocellulose having a viscosity as high as 1,000 seconds may be used, it is preferred to use a nitrocellulose of a 5 second grade or less. The only disadvantage of using a nitrocellulose of a higher viscosity is that the viscosity of the solution which is used to produce layer 13 is extremely high, rendering manipulation and preparation of the decorative strip difficult.

Regardless of the percentage of nitrocellulose in layer 13, and the grade of nitrocellulose, it is important to control the thickness of layer 13. Layer 13 should not be less than  $1 \times 10^{-4}$  inch, nor more than  $2 \times 10^{-4}$  inch in thickness. Using a grade of nitrocellulose of 5 seconds or less, an optimum thickness for layer 13 is  $1.5 \times 10^{-4}$  inch. Moreover, superior results are obtained, when higher grade viscosity nitrocellulose is used, if the thickness is limited to less than  $1.5 \times 10^{-4}$  inch.

The total thickness of layers 13 and 14 should be from  $4 \times 10^{-4}$  inch to  $6 \times 10^{-4}$  inch. When these thicknesses are exceeded the cohesion of layers 13

and 14 are so great that, when the carrier-backed decorative material has been applied to the surface formed by the edges of book sheets, or playing cards, the individual pages of books, or the individual playing cards, cannot be readily separated from each other without damage to the decorated surface. In the case of an embossed flat surface, exceeding these thicknesses results in such an increase in the cohesion of layers 13 and 14 that the lines of demarcation of the embossed areas are frequently ragged. When thicknesses less than these are used the adhesive qualities are so poor that the decorative material will not be properly adhered to the separated book sheet edges, playing card edges, or embossed surfaces.

Referring now more particularly to Fig. 2, there is shown a portion of an edge-decorated book sheet or playing card wherein 15 is a portion of 20 a book sheet or playing card, layer 14 is an adhesive, layer 13 is a mixture of nitrocellulose and adhesive, and layer 12 is the decorative material or metallic foil. The layers 13 and 14 are within the above-designated limits of thickness, and 25 layer 13 is composed of a mixture of nitrocellulose and adhesive within the above-designated percentage limitations.

In using this novel carrier-backed decorative film, the carrier-backed decorative strip, having 30 the adhesive incorporated therewith, is merely placed with the adhesive side down on a prepared surface, such as a flat leather surface, a cloth surface, the surface formed from any one of the 35 various materials commonly used for book coverings, or the smooth surface formed by the edges of playing cards or book leaves, assembled in side-by-side relation. Thereafter, heat or heat and pressure are applied to the carrier side of the 40 carrier-backed decorative material and the carrier is then removed, leaving the foil or decorative material firmly adhered to the prepared surface. In the case of playing cards or book leaves, the leaves or cards may then be rifled and separated, and when realigned they will 45 present a continuously decorated surface.

It should be apparent from the above description that there has been devised a novel and extremely useful carrier-backed decorative strip having incorporated therewith a material which, though not positioned exterior of the decorative 50 film when the decorative film is adhered to a surface, still results in the production of an abrasion-resistant decorative film. The use of such a combination results in revolutionary savings in time and labor in the edge-decorating of 55 playing cards or books, and enables the decorative material thereon, or on any embossed surface, to remain pleasing to the eye, even though subjected to the abrasion of normal use. The use of the carrier-backed decorative material described 60 herein will produce an abrasion-resistant decorative film which is as pleasing to the eye as a film placed on the edges of book sheets or playing cards by hand, and which has thereafter been 65 burnished.

While this invention has been described in its preferred embodiment, it is to be understood that the words that have been used are words of description rather than of limitation, and that changes within the purview of the appended 70 claims may be made without departing from the true scope and spirit of the invention.

What is claimed is:

1. A backed decorative material comprising a carrier, a release material on said carrier, a film

of decorative material on said release material, a film on said decorative material of a material comprising from 25% to 70% nitrocellulose and the balance polyamide adhesive, and a film of polyamide adhesive on said film of nitrocellulose-containing material; the thickness of said nitrocellulose-containing material film being from  $1 \times 10^{-4}$  inch to  $2 \times 10^{-4}$  inch, and the sum of the thicknesses of the nitrocellulose-containing material film and the film of polyamide adhesive being from  $4 \times 10^{-4}$  inch to  $6 \times 10^{-4}$  inch.

2. In a backed decorative material comprising a carrier, a release material on said carrier, a film of decorative material on said release material, and a film of polyamide adhesive, a film of a material comprising from 25% to 70% nitrocellulose and the balance polyamide adhesive on said film of decorative material and in intimate contact with said film of polyamide adhesive; said film of nitrocellulose containing material being from  $1 \times 10^{-4}$  inch to  $2 \times 10^{-4}$  inch, and the sum of the thicknesses of said polyamide adhesive film and said nitrocellulose-containing film being from  $4 \times 10^{-4}$  inch to  $6 \times 10^{-4}$  inch.

3. An edge-decorated book comprising a plurality of book pages, each of which said pages has in intimate contact with the edge thereof a layer of polyamide adhesive, said adhesive having in intimate contact therewith a layer of a material comprising from 25% to 70% nitrocellulose and the balance polyamide adhesive, and of a thickness of from  $1 \times 10^{-4}$  inch to  $2 \times 10^{-4}$  inch, said material having in intimate contact therewith a layer of decorative material, and the sum of the thicknesses of said nitrocellulose containing material and said polyamide adhesive being from  $4 \times 10^{-4}$  inch to  $6 \times 10^{-4}$  inch.

4. An edge-decorated playing card comprising a card, the edge of which has in intimate contact therewith a layer of polyamide adhesive, said adhesive having in intimate contact therewith a material comprising from 25% to 70% nitrocellulose and the balance polyamide adhesive, and being from  $1 \times 10^{-4}$  inch to  $2 \times 10^{-4}$  inch in thickness, said material having in intimate contact therewith a decorative material, the sum of the thicknesses of said nitrocellulose containing material and said polyamide adhesive being from  $4 \times 10^{-4}$  inch to  $6 \times 10^{-4}$  inch.

5. In a backed decorative material comprising a carrier, a release material on said carrier, a film of decorative material on said release material, and a film of polyamide adhesive, a film of a material comprising equal quantities of nitrocellulose and polyamide adhesives on said decorative material and in intimate contact with said film of polyamide adhesive; the thickness of said nitrocellulose containing film being from  $1 \times 10^{-4}$  inch to  $2 \times 10^{-4}$  inch, and the sum of the thicknesses of said nitrocellulose containing material and said polyamide adhesive film being from  $4 \times 10^{-4}$  inch to  $6 \times 10^{-4}$  inch.

6. In a backed decorative material comprising a carrier, a release material on said carrier, a film of decorative material on said release material, and a film of polyamide adhesive, a film of a material comprising equal quantities of nitrocellulose and polyamide adhesive on said decorative material and in intimate contact with said film of polyamide adhesive; the thickness of said nitrocellulose containing film being from  $1.5 \times 10^{-4}$  inch, the sum of the thicknesses of said nitrocellulose containing film and said polyamide adhesive film being  $5 \times 10^{-4}$  inch, and said nitrocellulose being of a 5 second grade.

7. In a backed decorative material comprising a carrier, a release material on said carrier, a film of decorative material on said release material, and a film of polyamide adhesive, a film of a material comprising from 25% to 70% nitrocellulose, of a grade of 1,000 seconds or less, and the balance polyamide adhesive, on said decorative material and in intimate contact with said film of polyamide adhesive; the thickness of said nitrocellulose containing film being less than  $1.5 \times 10^{-4}$  inch but not less than  $1 \times 10^{-4}$  inch, and the sum of the thicknesses of said nitrocellulose containing film and said polyamide adhesive film being from  $4 \times 10^{-4}$  inch to  $6 \times 10^{-4}$  inch.

8. An edge-decorated article comprising at least one sheet, the edge of said sheet having in intimate contact therewith a layer of polyamide adhesive, said adhesive having in intimate contact therewith a material comprising from 25% to 70% nitrocellulose and the balance polyamide adhesive, and being from  $1 \times 10^{-4}$  inch to  $2 \times 10^{-4}$  inch in thickness, said material having in intimate contact therewith a decorative material, the sum of the thicknesses of said nitrocellulose-containing material and said polyamide adhesive being from  $4 \times 10^{-4}$  inch to  $6 \times 10^{-4}$  inch.

WALLACE L. BOSTWICK.  
SAMUEL M. TERRY.

References Cited in the file of this patent

UNITED STATES PATENTS

| Number    | Name         | Date           |
|-----------|--------------|----------------|
| 1,124,114 | Davis et al. | Jan. 5, 1915   |
| 1,155,959 | Robinson     | Oct. 5, 1915   |
| 1,315,591 | Barker       | Sept. 9, 1919  |
| 1,515,676 | Grupe        | Nov. 18, 1924  |
| 1,515,722 | Boyd         | Nov. 18, 1924  |
| 1,591,304 | Giveans      | July 6, 1926   |
| 1,727,800 | Albert       | Sept. 10, 1929 |
| 1,909,631 | Poschel      | May 16, 1933   |
| 1,994,088 | Owen         | Mar. 12, 1935  |
| 2,017,367 | Kurz         | Oct. 15, 1935  |
| 2,099,641 | Bach         | Nov. 16, 1937  |
| 2,175,492 | Swift        | Oct. 10, 1939  |
| 2,285,178 | Thinius      | June 2, 1942   |